

Oct. 13, 1936.

J. D. BRADLEY

2,057,554

# METHOD OF AND APPARATUS FOR THE REDUCTION OF OXIDE ORES

Filed Aug. 3, 1932

4 Sheets-Sheet 1

*Fig. 1.*



## INVENTOR

INVENTOR  
James D. Bradley  
by his attorney  
Byrnes, Stettinius, Purnell and Blenko

Oct. 13, 1936.

J. D. BRADLEY

2,057,554

METHOD OF AND APPARATUS FOR THE REDUCTION OF OXIDE ORES

Filed Aug. 3, 1932

4 Sheets-Sheet 2

Fig. 2.



INVENTOR

James D. Bradley  
By his atto  
Byrnes, Robbins, Parmalee and Banks

Oct. 13, 1936.

J. D. BRADLEY

2,057,554

METHOD OF AND APPARATUS FOR THE REDUCTION OF OXIDE ORES

Filed Aug. 3, 1932

4 Sheets-Sheet 3

*Fig. 3.*



James D. Bradley  
by his atto  
Bynes, Stilbin, Sommerville and Block

Oct. 13, 1936.

J. D. BRADLEY

2,057,554

METHOD OF AND APPARATUS FOR THE REDUCTION OF OXIDE ORES

Filed Aug. 3, 1932

4 Sheets-Sheet 4

Fig. 4. B



Fig. 5.



INVENTOR

James D. Bradley  
by his atty  
Byrnes, Stibbs, Parmalee and Blenko

## UNITED STATES PATENT OFFICE

2,057,554

METHOD OF AND APPARATUS FOR THE  
REDUCTION OF OXIDE ORES

James D. Bradley, Pittsburgh, Pa.

Application August 3, 1932, Serial No. 627,340

20 Claims. (Cl. 75—91)

This invention relates to the recovery of metals from their ores, and more particularly to the recovery of metals wherein the ore is in the nature of an oxide either naturally or by conversion from its natural state to the oxide state.

Various attempts have been made to reduce ores, particularly iron ore, directly from the oxide to a metallic form without first reducing the ore in a blast furnace and then purifying the resulting metal in an open hearth or other purification furnace, but, for various reasons such methods have not proved to be highly practical from a commercial standpoint. Such methods as have heretofore been most successful have been characterized by the mixing of the ore with coal or coke and heating the mixture in a reducing atmosphere, the iron oxide giving up its oxygen to the adjacent carbon particles, leaving the iron in a metallic state. This is often referred to as "sponge iron".

The present invention is characterized by a method and apparatus in which the ore may be maintained out of contact at all times with solid reducing agents and in a reducing atmosphere which is highly reactive with the ore through the exclusion of atmospheric air. With the present invention the reduction is effected at a relatively low fuel cost per pound of metal secured and the practice of the invention yields combustible gas which may be employed for various purposes externally of the reducing plant.

The invention may be readily understood by reference to the accompanying drawings, which are more or less diagrammatic, and which are intended to merely show one embodiment of my invention, such details as are old and well-known in the art being omitted or only schematically illustrated.

In the drawings:

Figure 1 is a schematic view showing a side elevation of a complete plant for the practice of the invention;

Figure 2 represents a transverse vertical section through the retort and reducing apparatus detached from the various auxiliary equipment shown in Fig. 1;

Figure 3 is a staggered longitudinal vertical section substantially in the plane of line III—III of Fig. 2;

Figure 4 is a transverse horizontal section in the plane of line IV—IV of Fig. 3; and

Figure 5 is a detail view showing one arrangement for the melting of the processed ore.

According to the present invention, the ore to be treated is first preferably preheated and then introduced into a reducing chamber, preferably

of the type in which the ore is kept continuously agitated and in which the ore may move progressively from one end of the reducing chamber into the other. In this reducing chamber the ore, which is heated, but to a temperature insufficient to cause the melting of the iron, there is passed an atmosphere of highly reducing gases comprising coal gas ( $CH_4$ ), carbon monoxide ( $CO$ ), and hydrogen. These gases, before being introduced into the reducing chamber, are also heated. The  $CH_4$  component of the reducing gas combines with oxygen in the ore to form carbon dioxide ( $CO_2$ ) and water vapor ( $H_2O$ ). The carbon monoxide ( $CO$ ) combines with the oxygen of the ore to form  $CO_2$ , and the hydrogen gas combines with the oxygen of the ore to form water vapor. These reducing gases are generated in a retort, and the gases from the reducing chamber are returned to this retort. The retort is essentially a type of coking retort having a chamber in which coal, which incidentally may be a low grade coal, is introduced, and heat is applied from the exterior of the retort to the coal on the interior. The distillation of the coal yields hydrocarbon vapors, particularly the  $CH_4$ . As before stated, the spent gases, or partially spent gases, from the reducing chamber, are conducted from the reducing chamber to the retort, preferably into the bottom of the retort where the distillation of the coal has been pretty well completed and the coal reduced to a bed of glowing coke. Here, because of a deficiency of air, the system being closed against the admission of atmospheric air, the  $CO_2$  is broken down to form an increased volume of  $CO(C+CO_2=2CO)$ . The water vapor is broken down to form  $CO$  and hydrogen ( $H_2O+C=CO+H_2$ ). These gases formed in the hot coke bed of the retort mingle with the products of distillation from the green coal to produce the reducing atmosphere above described.

According to the preferred method of carrying out the process, the reducing gases, after leaving the retort, are cooled and treated to remove tar and sulphur and then forced by a compressor into a storage tank. Part of this gas is led from the storage tank to a preheater and after being preheated is introduced into the reducing chamber for contact with the heated ore. Another portion of this gas can be used to fire the retort. Still another portion of it may be used for melting the deoxidized ore to effect removal of slag and other contained impurities, and any further excess of the combustible reducing gas can be used as may be desired.

In carrying out this process, it will be observed,

first, that the ore and the carbonaceous reducing material do not come into contact except where the carbon is in a gaseous state. A second thing to be noticed is that the system is a substantially closed circulating system which excludes atmospheric air. The reducing gases, therefore, are not diluted with atmospheric nitrogen, with the result that they have a much higher affinity for the oxygen of the ore, it being well understood that dilution with inert substances reduces the rapidity and the efficiency of most chemical reactions.

In carrying out the method, I prefer that the system be operated at a pressure above atmospheric pressure, say a pressure of one atmosphere, so as to exclude atmospheric air, and because of this pressure and the fact that the gases are not diluted with nitrogen, the efficiency of the process is further increased.

20 A further point of merit in the system is the manner in which available heat units are used, with the result that the ore may be reduced at a relatively low fuel cost. In this connection it may be pointed out that the preheating of the reducing gas after it leaves the storage tank can be accomplished, and in the preferred practice of the invention, is accomplished by utilizing excess heat from the retort. In like manner excess heat from the retort is utilized in maintaining the ore at the reaction temperature and for preheating the ore. The heat from the reducing gases and products of distillation from the retort may be used for generating steam to supply the retort where additional water vapor is desirable.

35 In the process, the deoxidized ore may be obtained in its divided form and used in such commercial operations as require a sponge iron of this nature. For the production of metals, however, the process further contemplates the introduction of the treated ore, preferably before it loses its heat, into a bath of molten metal and preferably in a state of diffusion, together with reducing gases, whereby any particles that have been only partially deoxidized may be completely deoxidized in this bath. The slag forming impurities are released from the particles and float to the top of the metal while the metal may be tapped from time to time from the bottom of the bath.

50 Because of the fact that the process may be carried out without bringing the ore into contact with solid carbon particles, those impurities of coal and coke which form the ash of coal or coke are not mixed with the ore, with the result that 55 the metal is not contaminated from the fuel and the metal which results is very low in carbon, and, moreover, the bulk of reduced ore does not have to be treated for the removal of carbon and coal or coke ashes. Since, moreover, the process may 60 be effected without having the coal or coke in contact with the ore, the ore itself may be brought more rapidly to the reaction temperature than where there is a relatively large mass of comminuted coal or coke and comminuted ore, all of 65 which has to be heated to the reaction temperature. The reaction temperature with high grade ores can also be higher because of the absence of those slagging impurities provided by coal or coke. This is desirable because the reaction of 70 course takes place more effectively when the ore is highly heated, and it also takes place where the particles of the ore do not tend to cling together and agglomerate as they do if the temperature is too high and there are too many slag 75 forming ingredients present.

The process may be further and better understood and the novel apparatus will be described by reference to the accompanying drawings. Referring first to Fig. 1, A designates the retort or reducing gas producing unit and B designates the ore treating unit. The letter C designates the melting. The various gas treating and gas storage units of the system are designated generally as D.

The unit A, shown in more detail in Figs. 2 10 and 3, comprises an outer wall structure 2 within which is a retort 3 having a distillation chamber 4. The walls 2 of the structure are preferably formed of a heat insulating refractory, while the retort walls 3 are preferably formed of a heat 15 conducting refractory such as silicon carbide. In the bottom of the unit A is a pit 5 adapted to hold a body of water 6, and the lower end of the retort 3 projects into this pit so as to be sealed by the water. It is supported on piers 7 at its 20 bottom. It is also provided with an ash pan 8 having a screw conveyor 9 therein for the removal of ashes from the bottom of the retort. In the retort above the water line there is a grate 10 for supporting the coal and coke in the distillation chamber 4. The walls of the retort 3 are spaced inwardly from the outer walls 2 in order to provide a combustion space 11 at each side of the retort. The combustion spaces 11 are closed at their bottoms above the level of the wall 30 seal by refractory partitions 12. The retort 3 is of a generally rectangular shape, the combustion spaces 11 being provided only at opposite sides of the retort, while the ends of the retort are closed by the refractory walls 13, as shown in 35 Fig. 3.

Located near the lower ends of the combustion spaces 11 are gas burners 14. At the top of the retort 3 there is a roof 3a, and this roof has one or more extensions 3b projecting through the 40 top 15 of the unit A. Mounted above these extensions are feed hoppers 3c having feed chutes 3d delivering into the extensions 3b and provided with the conventional bell type closures 3e for permitting the material to be fed from the hoppers into the retort while sealing the retort against the escape of gases through the hoppers. 45

The unit B for the deoxidation of the ore comprises a refractory structure which is above the unit A and offset laterally with respect thereto. 50 As illustrated, it has side walls 16 and end walls 17 which enclose a vertical chamber 18. Leading from the top of the unit A is a flue passage 19 that opens into the bottom of the chamber 18. The chamber 18 is provided with a refractory baffle 20, the arrangement being best shown in Fig. 3 where it will be noted that the passage 19 opens into the chamber 18 at one side of the chamber. The baffle 20 divides the interior chamber into a lower passage 18a and an upper compartment 18b. The baffle 20 has an opening at 21 at that end which is opposite the flue 19 so that the gases from the unit A flow first along the passage or compartment 18a, then through the port 21, and in the opposite direction along 65 the upper compartment 18b. In the upper part of the compartment 18b there are two heat exchangers placed side-by-side and designated 22 and 23. They are of sheet metal construction, being formed of a heat resistant metal. 70

At the end opposite the baffle opening 21 these heat exchangers provide a vertical passage 24 between them so that the gases entering the compartment 18b through the port 21 flow longitudinally through this compartment into the ver- 75

tical port or passage 26. The passage 26, in turn, opens into a horizontal passage 28 formed between upper and lower parts of the two exchanger units 22 and 23. This horizontal passage in turn 5 terminates in a vertical passage 29 leading to a stack 27.

In the upper compartment 18b there is an ore preheater which may conveniently comprise a heat resisting metal cylinder 28 having a receiving spout 29 at one end thereof which is turned upwardly and which communicates with a feed chute 30 leading from a hopper 31, the chute 30 being provided with feeding bells 32 of the conventional type, permitting the ore to 10 be fed into the preheater 28 while preventing the escape of gas from this unit. At the opposite end of the drum 28 is a downwardly turned discharge pipe 33 and in the drum 28 is a screw conveyor 34 for progressively moving the incoming ore from one end of the drum to the other. The ore discharging from the outlet 33 delivers 15 into the inlet extension 35 of the reducing chamber, which is in the lower compartment 18a of the chamber 18, and which is designated 36. 20 This reducing chamber may conveniently comprise a drum formed of heat resisting metal having a screw conveyor 37 therein for agitating the ore and for causing it to travel from one end 25 of the drum to the other, although obviously any other suitable agitating and conveying means 30 may be used.

On the end of the drum 36 opposite the intake 38 is a discharge pipe 39. The screw conveyors 34 and 37 may be operated by common gearing 35 which, in turn, is geared to a driving motor 39.

Referring again to Fig. 1, the distillation chamber of the retort has one or more outlet pipes 40 leading from a point near the top of the distillation chamber and preferably above the normal coal level in the retort. This pipe 40 conveys the gases from the retort to a cooler or heat exchanger 41 which is conventionally illustrated and which may be of any well-known type. I have shown a heat exchanger in which there is 45 a water boiler 42 by means of which the gases from the retort can heat water to generate steam, the boiler having an inlet pipe 43 and a steam outlet pipe 44. The heat exchanger 41 has a gas discharge pipe 45 leading to a tar extractor 50 46 of any known or preferred construction, and which is only conventionally illustrated, such elements being well-known in the coal distillation industry and forming no part of the present invention. From the tar extractor the gases are 55 passed through pipe 47 to a desulphurizer 48, which is also conventionally illustrated, being a device well-known and commonly employed in the coal distillation industry, which serves to remove sulphur containing products from the gases. 60 The gas is now cooled sufficiently so that it can be handled by a compressor. Leading from the desulphurizer 48 there is a pipe 49 which goes to a compressor 50, the compressor being conventionally illustrated. The compressor discharges 65 into the storage tank 51. The pressure storage tank 51 has a gas outlet passage 52 coupled into a line 53. One branch of this line leads through a pressure regulator conventionally indicated at 54, to a circulating pump 55. 70 Leading from the circulating pump 55 is a pipe 56 which goes into the top of the heat exchanger unit 23. Leading from the bottom of the heat exchanger unit 23 is a pipe 57 which opens into the reducing drum 36 (see Fig. 3).

75 By reason of this arrangement the reducing

gas from the storage compartment is preheated in the preheater 28 and then discharged in its heated state into the ore reducer where it travels through the ore in a direction counter to the direction of movement of the ore and while the ore is being constantly stirred and agitated. These gases, upon leaving the reducer, enter the ore preheating unit 28, again traveling through the ore in a direction counter to the flow of the ore, and they are removed from the unit 28 through pipe 58. The pipe 58 (see Fig. 1) opens into the distillation chamber 4 of the retort above the grate 18, at the point designated 59, in Figs. 2 and 3. The steam pipe 44 may join to the pipe 58, as shown in Fig. 1, so that steam can 15 be introduced into the retort along with the spent reducing gas.

The burners 64 are connected by a pipe 60 through which a combustible mixture is supplied to them. The pipe 60 may have a branch 61 20 leading to any suitable gas generator (not shown) for supplying gas in the initial operation of the system. After the system has been operated and gas is available from the storage tank 51, it may be conveyed to the pipe 60 through pipe 62, and 25 blower 63. The blower is designed to handle a mixture of gas and air, and the air is supplied through pipe 64 leading from the preheater unit 22. The air enters the preheater unit 22 from 30 atmosphere.

The deoxidized ore discharging from the outlet 38 of the unit 36 may be conveniently carried directly through a pipe or chute 65 into the unit C which may be arranged as shown in Fig. 1 for the ore to go into the bottom of the unit, being 35 blown in by a blast of reducing gas supplied through pipe 66 and pump 67 which is connected to the pipe 62. This unit C is heated from the burners 68 arranged around the top of the unit C and supplied from the manifold 69 connected to 40 a pipe 70 with the pipe 60 so as to receive the combustible mixture from the blower 63. Preferably, however, the unit C is of the construction shown in Fig. 5 in which the chute 65' has a feeder 71 therein of any preferred or conventional type. 45 I have shown the feeder 71 as comprising a valve-like body having a plurality of pockets operating within the chamber. This permits the material to be fed down the chute 65' without any substantial up-draft of gas from the unit C. 50

The chute 65', as shown in Fig. 5, discharges into the top of the unit C, which comprises a refractory structure 72 having a chamber 73 therein. In the chamber 73 and projecting through the top thereof is a refractory casing or well 74 55 into which the chute 65' discharges. This well or casing extends down into the chamber to a point adjacent the bottom thereof. The burners 68 serve to heat the interior of the structure and enter the structure through the top thereof. 60

At the bottom of the structure there is a port 75 through which metal may be drained from time to time and which may be sealed at other times by a refractory plug, as shown. Spaced above the floor of the melting chamber there is another 65 opening or port 76 through which slag may run off when the metal and slag reaches a predetermined depth in the melting chamber.

Opening into the well or casing 74 at the top of the melting chamber is a pipe 66' corresponding 70 to pipe 66 shown in Fig. 1, and which leads to a source of reducing gas. Burned gases are led out of the chamber 73 through a flue 77.

The operation of the system may now be followed. Coal is charged from the hopper 3c into 75

the coking retort until the retort is nearly full. As previously stated, the operation permits of the use of an inferior grade of coal where this is the cheapest material obtainable. The invention also makes it commercially practicable to use a low grade of ore. Heat is applied to the retort through the combustible mixture introduced into the chamber 11 through the burners 14. The heat of this combustion is transmitted through the walls of the retort to effect distillation of the coal while the highly heated gases are conducted from the combustion chambers 11 through the passage 19 and to the lowermost compartment 18a of the chamber 18. They flow along this compartment, heating the ore reducing chamber 36, then flowing along the upper compartment 18b, preheating the ore in the preheater 28. From this point they flow through the heat exchangers 22 and 23, heating the air for combustion in the heat exchanger 22 and heating the reducing gases for the reduction of the ore in the heat exchanger 23. The gases from the retort, on the other hand, pass through the pipe 40 into the heat exchanger 41, where they are cooled, thence to the tar remover, and from there into the desulphurizer, after which they are forced by the compressor into the storage tank 51. From the storage tank some of these gases are led to the burners 14. Other gas is led to the heat exchanger 23 and from the heat exchanger through the pipe 57 into the reducing unit 36. Here the reducing gases flowing across and through the heated ore react with the ore to remove oxygen from the ore. Leaving the reducing unit, they are conducted through the ore preheating unit 28 where they may have some effect in the initial reduction of the ore. They are removed from the ore preheater and conducted through the pipe 58 back to the bottom of the retort. After a period of operation the retort contains a bed of glowing coke in the lowermost zone thereof. As previously explained, the spent gases from the ore reducing unit, comprising principally carbon dioxide and water vapor, are broken up to form carbon monoxide and free hydrogen. Carbon monoxide and free hydrogen together with hydrocarbon gas which is driven off from the distribution of the coal comprises the reducing gas which is circulated through the reducing unit 36, the gases having been cleaned of tar and sulphurous compounds before being introduced into the reducing unit.

There is thus maintained a closed circulation of gases from the retort to the reducing unit and back to the retort, with the result that atmospheric air is not drawn into the system and the reducing gases are thus not diluted. Since there is a constantly increasing volume of gas being generated through the conversion of carbon dioxide and water vapor generated in the ore reducing unit to carbon monoxide and hydrogen, plus additional gases of distillation in the retort, an excess of gas is available for the burners 14 and 68.

65 The ore, after it has been deoxidized, discharges into the unit C through the central well or casting 14 into which there is being blown at the same time a volume of the reducing gas. The ore particles are thus again brought into intimate contact with reducing gas and are heated from the burners 68 at the same time. There is preferably at all times a residuum of molten metal in the bottom of the chamber 13 which accelerates the melting of the ore particles with the 70 liberation of entrapped slag and impurities. In

75 this final diffusion of the reducing gas and the heated ore particles in the presence of the molten metal, particles which have not been completely deoxidized are thereby completely deoxidized.

An important advantage of bringing the treated ore into intimate contact with molten metal, or blowing it through the molten metal, is that the fines and dust-like particles are immediately and completely absorbed, whereas in the ordinary 10 ore reducing processes the fines are blown out as fine dust.

The metal which accumulates in the unit C, which is tapped off from time to time to be cast 15 into molds, or to be further treated, as may be desired, has been found to be of a very pure quality, low in carbon, and low in those impurities which are normally found in pig iron from blast furnaces.

20 While I have, in the foregoing description, mentioned iron ore specifically, the invention is not confined to the reduction of oxides of iron, but is applicable to the reduction of various other metallic oxides. Due to the concentration of the reducing gases and the exclusion of inert gases, 25 the reducing operations are effected at temperatures considerably below those at which it has heretofore been thought practical to reduce ores, which is an advantage not only from the standpoint of the heat saved, but from the fact that 30 the equipment and refractories are not disintegrated so rapidly at the lower temperatures at which the process can be effected. It is for the same reason that ores of other metals than iron, such for instance, as chromium, have been 35 successfully reduced to a metallic state with this process.

Where the ore is a sulphide ore, or contains 40 a percentage of sulphide, the sulphur will combine with the reducing gas. In such instances, it may be necessary to circulate the spent reducing gas through water or other treating apparatus to absorb any sulphuric or sulphurous acids that are formed before the gases are returned to the 45 retort.

It will also be appreciated that while I have described in considerable detail one specific system with particular apparatus that various changes and modifications may be made in the construction and disposition of the various parts 50 within the contemplation of my invention and under the scope of the following claims.

I claim:

1. The herein described method which comprises heating a retort containing a body of coal 55 to effect distillation of the coal, utilizing excess heat from such heating operation to heat a mass of ore, circulating the gases from the retort over the heated ore, and then returning them to the retort and reducing them.

2. The herein described method which comprises heating a retort containing a body of coal to effect distillation of the coal, utilizing excess heat from such heating operation to heat a mass of ore, circulating the gases from the retort over 60 the heated ore, then returning them to the retort and reducing them, and cooling, cleaning and again heating the gases after they leave the retort and before they are brought into contact with the heated ore.

3. An apparatus of the class described comprising a retort, a combustion chamber around the retort, an ore reducing unit outside the combustion chamber, means for conveying hot gases of combustion from the combustion chamber to the 75

- exterior of the reducing unit for heating the same, means for circulating gases from the retort to the reducing unit, and means for conveying gases from the reducing unit back to the retort.

4. An apparatus of the class described comprising a retort, a combustion chamber around the retort, an ore reducing unit, means for conveying hot gases of combustion from the combustion chamber to the exterior of the reducing unit for heating the same, means for circulating gases from the retort to the reducing unit, and means for conveying gases from the reducing unit back to the retort, said reducing unit comprising a chamber having means for agitating the ore.

15 5. An apparatus of the class described comprising a retort, a combustion chamber around the retort, an ore reducing unit, means for conveying hot gases of combustion from the combustion chamber to the exterior of the reducing unit for heating the same, means for circulating gases from the retort to the reducing unit, means for conveying gases from the reducing unit back to the retort, said reducing unit comprising a drum having means for receiving the ore at one end, 20 means for discharging the ore at the other end, and means for conveying the ore therethrough from one end to the other.

25 6. An apparatus of the class described comprising a retort, a combustion chamber around the retort, an ore reducing unit, means for conveying hot gases of combustion from the combustion chamber to the exterior of the reducing unit for heating the same, means for circulating gases from the retort to the reducing unit, means 30 for conveying gases from the reducing unit back to the retort, said reducing unit comprising a drum having means for receiving the ore at one end, means for discharging the ore at the other end, means for conveying the ore therethrough from one end to the other, an ore preheating 35 unit also heated from the gases of combustion and out the retort and comprising an enclosed chamber having conveying means therein, one end of the preheating unit discharging into the receiving end of the reducing drum, and means for feeding ore into the other end of the preheating unit, said feeding means including means for preventing the free escape of gas from the ore preheating unit.

40 7. An apparatus of the class described comprising a system having a retort, an ore reducing unit, a common means for heating the retort and the ore reducing unit, means for conveying gases from the retort to the ore reducing unit, means for returning gases from the ore reducing unit to the retort, said system comprising the retort and ore reducing unit being substantially closed against the introduction of atmospheric air, the means for conveying gases from the retort to the ore reducing unit including a heat exchanger, a gas cleaning means, a compressor, a storage tank, and a gas preheater between the storage tank and the ore reducing unit.

45 8. An apparatus of the class described comprising a system having a retort, an ore reducing unit, a common means for heating the retort and the ore reducing unit, means for conveying gases from the retort to the ore reducing unit, means for returning gases from the ore reducing unit to the retort, said system comprising the retort and ore reducing unit being substantially closed against the introduction of atmospheric air, the means for conveying gases from the retort to the ore reducing unit including a heat exchanger, a 50 gas cleaning means, a compressor, a storage tank, and a gas preheater between the storage tank and the ore reducing unit.

55 9. Apparatus for the reduction of metal from ore, comprising an ore reducing unit, means for circulating reducing gas through the unit, including a gas generator, the reducing unit being substantially closed against atmospheric air, means for conveying reduced ore from the ore reducing unit to a melting unit and terminating below the normal level of molten metal in the melting unit, and means for mixing reducing gas in intimate contact with the deoxidized ore before the reduced ore has been completely melted.

60 10. An apparatus of the class described, comprising a melting receptacle having burners therein, a common conduit through which reducing gas and comminuted ore are introduced into said receptacle, said conduit terminating adjacent the bottom of the melting unit an ore deoxidizing unit closed against the free circulation of air therethrough discharging into said conduit, means for circulating heated reducing gases through said deoxidizing unit, and means in the deoxidizing unit for agitating the ore and conveying it to the conduit.

15 11. A system of the class described comprising an ore reducing unit having means for continuously conveying ore therethrough, means for feeding ore to said unit while substantially excluding the escape of gas therefrom, a retort, means for continuously supplying coal to the retort, a combustion chamber outside the retort, means for conveying gases from the combustion chamber around the reducing unit to heat the ore in the reducing unit, a gas cleaning and storage system into which the gases from the retort are passed, means for receiving gas from the cleaning and storage system, preheating it and conveying it to the reducing unit, said reducing unit being substantially closed against the escape of gases to the atmosphere, and means for conveying the gases from the reducing unit back to the retort.

20 12. A system of the class described comprising an ore reducing unit having means for continuously conveying ore therethrough, means for feeding ore to said unit while substantially excluding the escape of gas therefrom, a retort, means for continuously supplying coal to the retort, a combustion chamber outside the retort, means for conveying gases from the combustion chamber around the reducing unit to heat the ore in the reducing unit, a gas cleaning and storage system into which the gases from the retort are passed, means for receiving gas from the cleaning and storage system, preheating it and conveying it to the reducing unit, said reducing unit being substantially closed against the escape of gases to the atmosphere, means for conveying the gases from the reducing unit back to the retort, burners in the combustion chamber for heating the retort, and means for conveying gases from the cleaning and storage system to said burners.

25 13. A system of the class described comprising an ore reducing unit having means for continuously conveying ore therethrough, means for feeding ore to said unit while substantially excluding the escape of gas therefrom, a retort, means for continuously supplying coal to the retort, a combustion chamber outside the retort, means for conveying gases from the combustion chamber around the reducing unit to heat the ore in the reducing unit, a gas cleaning and storage system

into which the gases from the retort are passed, means for receiving gas from the cleaning and storage system, preheating it and conveying it to the reducing unit, said reducing unit being substantially closed against the escape of gases to the atmosphere, means for conveying the gases from the reducing unit back to the retort, burners in the combustion chamber for heating the retort, means for conveying gases from the cleaning and storage system to said burners, and means heated by gases from said combustion chamber for pre-heating air and supplying it to said burners.

14. The method of reducing ore which comprises agitating the ore in a receptacle substantially closed against atmospheric air, heating the ore while it is being agitated, passing a reducing gas substantially free of atmospheric air through the chamber during heating and agitation of the ore, thereafter reducing any gases which have been oxidized by contact with the ore and recirculating them, and enriching the gases so circulated with additional hydrocarbon gases.

15. An ore-reducing and gas-generating apparatus comprising an externally heated gas producing retort, a reducing unit where gas and oxygen-containing ore are brought into intimate contact, means including gas cooling, cleaning and storing equipment for conducting gas from the retort to the reducing unit, means for reheating the gas before it enters the reducing unit after leaving the storing equipment, and means for conveying spent gas from the reducing unit back to the retort.

16. The method of reducing ore and generating gas which comprises subjecting a mass of carbonaceous material to heat and generating a reducing gas therefrom, cooling and storing the reducing gas, conveying some of the gas which has been cooled into intimate contact with a mass of heated oxygen-bearing ore to reduce the ore, returning the used gas to the heated carbonaceous mass, maintaining the gases and the carbonaceous mass and the ore during the operation substantially out of contact with atmospheric air, and utilizing waste heat from the heating of the carbonaceous mass for supplying heat to aid in reducing the oxygen-containing ore.

17. The method of treating ore to recover metal therefrom, which comprises subjecting the ore to the action of a reducing gas and out of contact with solid carbonaceous material and at

a temperature below which appreciable melting of the resulting metal particles takes place, then discharging the treated ore into a molten metal and slag bath below the surface of said bath, and simultaneously discharging a reducing gas into the bath below the surface thereof to further react on unreduced ore particles, the metal in said bath comprising metal recovered from the ore.

18. The method of treating ore to recover metal therefrom, which comprises subjecting the ore to the action of a reducing gas and out of contact with solid carbonaceous material and at a temperature below which appreciable melting of the resulting metal particles takes place, then discharging the treated ore into a molten metal and slag bath below the surface of said bath, and simultaneously discharging a reducing gas substantially free of atmospheric nitrogen into the bath below the surface thereof to further react on unreduced ore particles, the metal in said bath comprising metal recovered from the ore.

19. Apparatus for the reduction of ore and generation of gas, comprising a gas producer and an ore-reducing unit and a gas circulating system connecting the two and arranged to transfer gas from the producer to the ore-reducing unit and from the ore-reducing unit back to the producer, the entire system being substantially closed to entrance of atmospheric air, the system including means for cooling and storing the gas after it leaves the producer and before it is returned to the reducing unit and for reheating it by waste heat from the producer after it leaves the storing means and before it enters the reducing unit.

20. Apparatus for the reduction of ore and generation of gas, comprising a gas producer and an ore-reducing unit and a gas circulating system connecting the two and arranged to transfer gas from the producer to the ore-reducing unit and from the ore-reducing unit back to the producer, the entire system being substantially closed to entrance of atmospheric air, the system including means for cooling and storing the gas after it leaves the producer and before it is returned to the reducing unit, the producer being of the heated retort type, and means whereby excess heat from the producer is utilized in the reducing unit.

JAMES D. BRADLEY.